

## UNITED STATES PATENT OFFICE

2,062,977

PROCESS OF PRODUCING ALUMINUM  
ALLOY RIVETSSven E. Hybinette and Justin E. Tingay, Jackson,  
Mich., assignors to The Nicalumin Company,  
Jackson, Mich., a corporation of MichiganNo Drawing. Application February 23, 1934,  
Serial No. 712,484

14 Claims. (Cl. 148—11.5)

The present invention relates to improvements in aluminum alloy rivets and the process of producing the same.

Aluminum alloy rivets that are in use at the present time are made from duralumin alloys containing considerable quantities of copper and silicon, and are, therefore, subject to spontaneous aging. As a consequence, such rivets are made from annealed or cold worked wire and the consumers have to quench the rivets within one hour before using them. An improvement has recently been made in this practice whereby the quenched rivets are held at a low temperature so as to retard the spontaneous aging. However, all practices, up to the present development, have necessitated the requenching of the rivets from time to time so as to make sure that heading up of the rivet is made before any considerable age hardening has taken place. Obviously, any procedure which is so dependent upon the time element between quenching and heading of the rivet is uncertain and unreliable and it is a well known fact that airplane, zeppelin, bus and truck structures have heretofore suffered from so-called "popping" of rivets, or in other words, the heads of the aluminum alloy rivets fall off. This failure of riveted structure is mainly attributable to age hardening before heading up of the rivet. Under present practice, satisfactory fabrication rests entirely upon the workman's judgment as to the lapse of excessive time between the quenching and the riveting operation rendering the rivets unfit for use without requenching. In all events, the original head of the rivet is much softer than the finally headed up end of the rivet.

Generally, it becomes the object of the present invention to provide aluminum alloy rivets which obviate the above objections and disadvantages and to produce rivets which are equally strong in both ends, which are more reliable and even in quality and which are not subject to the workman's opinion of whether they are too hard or not, at the time of the riveting operation, to give a satisfactory joint.

More specifically, the present invention has for one of its objects to provide an artificially aged aluminum alloy rivet of such stable characteristics as to permit the use of the same, with substantially uniform results, an indefinite period after heat treatment. Another object is to provide aluminum alloy rivets characterized by having both heads thereof of approximately the same hardness. A further object is to do away with the necessity of having a heat treating

operation in every riveting shop. These and other objects of the invention will be more fully set forth in the description to follow.

In carrying out the invention, alloys which age spontaneously cannot be used. For this reason the copper content must be held within a definite range. Furthermore, high silicon alloys are not desirable because of the excessive hardness imparted by the heading up of the already aged rivet. For these reasons, alloys of the copper-silicon-magnesium, copper-silicon, or silicon-magnesium type have not been found suitable. Best results have been obtained with alloys of the type disclosed in United States Patent No. 1,579,481. Other alloys may be found useful as long as they fill the main requirements of being ductile enough after complete aging to produce a sound rivet and the composition of the metal is such as not to be subject to more than a very slight aging at ordinary temperatures.

By way of an example, an alloy containing approximately .5% to 1% nickel, .1% to 1% copper, .25% to .5% chrome group metals and/or manganese with about 1/2% magnesium has been found to be satisfactory. No silicon and iron is added in the alloy except such quantities as enter into the alloy as so-called impurities. That is to say, there may be present about 1/2% each of iron and silicon. It is to be understood that the composition can be varied and changed within the limits of physical properties hereinbefore mentioned, and within the limits of the claims.

The alloys coming within the type disclosed in the aforesaid patent must be composed in such a way as to have the required plasticity of the rivet even in their fully heat treated state. They are peculiar in that they only acquire a strength fully comparable to that of duralumin if they are cold worked or stress hardened after quenching and/or after aging. Without such work hardening they are too soft. It is evident that the heads of a rivet get this required work hardening but the shank of the rivet is not work hardened to the same extent as the heads and, therefore, not so strong. The shank is subjected to shearing stress and it has heretofore been understood that strength in shear always is in a certain relation to tensile strength. However, we have found that such is not the case with these alloys when the work hardening is produced by rolling or drawing but it is the case when the work hardening consists in compression or upsetting. It is, therefore, evident that to give the shank the required strength it must be up-

set. This upsetting of the shank is to a certain extent accomplished in a rivet producing machine because the hole in the die must always be somewhat larger than the wire from which the rivet is made. If the wire is of too small diameter the head comes eccentric on the shank. In ordinary practice such upsetting amounts only to from one to three per cent difference in diameter between the original wire and the finished rivet. Another upsetting is made in the final closing up of the rivet because the hole is generally made somewhat larger in diameter than the shank of the rivet. The total upsetting of the rivet is, therefore, in maximum a 6% increase in diameter. For many purposes this upsetting is enough but when it comes to rivets for aircrafts and automobiles, greater strength is required. As will be hereinafter described, we have found means of increasing the upsetting in the rivet making by departing from conventional circular wire section. It may be done by upsetting the shank in a special die simultaneously with the making of the rivet or before or after the head is formed, but a more convenient way is to use polygon shaped wire and one operation. In this way we are able to produce rivets which are superior in shearing strength to any aluminum alloy rivets that we know of.

The process of fabrication of aluminum alloy rivets which, according to the present invention, overcomes the hereinbefore enumerated objections, consists in the following steps. An alloy of the type stated is selected which is suitable for the purpose. The alloy is drawn to wire of the desired dimension. At this point a departure from prior practice is preferably made; in lieu of being of circular section, the wire is preferably of regular polygonal section and may be square, hexagonal, octagonal, etc., depending upon the amount of work hardening that is desired. After drawing, the wire is quenched in the ordinary way, well known to those versed in the art. This wire may, or may not be, slightly work hardened by drawing or stretching after quenching. Rivets are then made from this wire in the ordinary rivet making machines. It is to be understood that the wire of regular polygonal section will center itself in the usual circular hole in the die of the riveting machine; then upon upsetting the rivet head, the shank of the rivet will also be upset in the die to the extent required to fill the die and impart the circular contour of the die to the rivet shank. In this manner every desired degree of work hardening is produced in the shank of the rivet. The completed rivets are then aged at an elevated temperature, usually about 300° Fahrenheit, and this aging temperature, as well as the time of aging, is adjusted and controlled according to the analysis of the alloy and according to the work hardening that has been given to the shank so as to produce a rivet that can be headed up without becoming too hard or brittle, in other words a rivet of the most desirable temper.

The foregoing process may be considered as comprising the following general steps in its execution: (a) Selection of an aluminum alloy not subject to much spontaneous aging and plastic enough even after a work hardening in connection with the heat treatment. (b) Making wire of such alloy of shape and dimension to enable work hardening of the rivet shank in the die of the rivet machine due to upsetting. Such work hardening in round wire is only possible to the extent of a few per cent, because the wire must

be held near and centered in the hole of the die. Our preferred wire section is hexagonal with fairly well rounded corners. It is evident that the same results may be obtained by other ways of upsetting the metal in the shank and we do not wish to limit our invention to the use of polygon-shaped wire for such purposes. (c) Quenching or subjecting the wire to a solution heat treatment. (d) Producing the rivet in a rivet making machine provided with means for upsetting of the shank. (e) Aging the rivets with control of aging temperature and time of aging in such a way that rivets of the correct temper are produced.

We claim:

1. The process of manufacturing rivets from aluminum alloys susceptible to heat treatment comprising forming a wire of non-circular cross-section, upsetting said wire to form rivets having shanks of cross-section greater than the wire, said shanks being upset within a circular die to impart a circular cross-section to the shanks.

2. The process of manufacturing rivets from aluminum alloys which comprises forming a head on a wire of polygonal cross-section and upsetting the wire to form a shank of circular cross-section.

3. The process of manufacturing rivets from artificially aging aluminum alloys characterized by their low silicon content and non-spontaneous aging comprising making the rivets from quenched wire, the shanks of such rivets having a cross-section greater than that of the wire, said greater cross-section being produced by upsetting while cold, and producing such a temper by aging at a predetermined temperature for a predetermined time according to the analysis of the alloy, that the rivets may be headed up without becoming too brittle.

4. The process of manufacturing rivets from artificially aging aluminum alloys characterized by their low silicon content and non-spontaneous aging comprising making the rivets from quenched wire, work hardening the shanks thereof by upsetting cold and producing such a temper by aging at a predetermined temperature for a predetermined time according to the analysis of the alloy, that the rivets may be headed up without becoming too brittle.

5. The process of manufacturing rivets from artificially aging aluminum alloys characterized by their low silicon content and non-spontaneous aging comprising the making of rivet blanks from quenched wire, upsetting the same while cold, making rivets from such upset blanks and producing such a temper by aging at a predetermined temperature for a predetermined time according to the analysis of the alloy, that the rivets may be headed up without becoming too brittle.

6. The process of manufacturing rivets from artificially aging aluminum alloys characterized by their low silicon content and non-spontaneous aging comprising the making of wire of a polygonal cross-section, quenching the same, making rivets from such quenched wire, such rivets having shanks of substantially greater cross-sectional area than said wire, said greater cross-section being produced by upsetting while cold, said upsetting being within a circular die to impart a circular cross-section to the shanks, and producing such a temper by aging at a predetermined temperature for a predetermined time according to the analysis of the alloy, that the rivets may be headed up without becoming too brittle.

7. The process of manufacturing rivets from artificially aging aluminum alloys characterized

by their low silicon content and non-spontaneous aging comprising over 92% aluminum, .5% to 1% of nickel, .1% to 1% of copper, .25% to .5% chrome group metals and/or manganese and 5 about .5% magnesium, which comprises the making of rivets from quenched wire, the shanks of such rivets having a cross-section greater than that of the wire, said greater cross-section being produced by upsetting while cold, and producing 10 such a temper by aging at a predetermined temperature for a predetermined time according to the analysis of the alloy, that the rivets may be headed up without becoming too brittle.

8. The process of manufacturing rivets from 15 artificially aging aluminum alloys characterized by their low silicon content and non-spontaneous aging comprising over 92% of aluminum, 5% to 1% of nickel, .1% to 1% of copper, .25% to .5% chrome group metals and/or manganese and 20 about .5% magnesium, which comprises the making of rivets from quenched wire, work hardening the shanks thereof by upsetting cold and producing such a temper by aging at a predetermined temperature for a predetermined time according 25 to the analysis of the alloy, that the rivets may be headed up without becoming too brittle.

9. The process of manufacturing rivets from artificially aging aluminum alloys characterized by their low silicon content and non-spontaneous 30 aging comprising over 92% of aluminum, .5% to 1% of nickel, .1% to 1% of copper, .25% to .5% chrome group metals and/or manganese and about .5% magnesium, which comprises the making of rivet blanks from quenched wire, upsetting 35 the same while cold, making rivets from such blanks and producing such a temper by aging at a predetermined temperature for a predetermined time according to the analysis of the alloy, that the rivets may be headed up without becoming too brittle.

10. The process of manufacturing rivets from artificially aging aluminum alloys characterized by their low silicon content and non-spontaneous aging comprising over 92% of aluminum, .5% to 45 1% of nickel, .1% to 1% of copper, .25% to .5% chrome group metals and/or manganese and about .5% magnesium, comprising forming a wire and upsetting said wire to form a rivet having a shank which has at least a 5% greater area of 50 cross-section than said wire from which the rivet is formed.

11. The process of manufacturing rivets from

artificially aging aluminum alloys characterized by their low silicon content and non-spontaneous aging comprising the making of rivets from quenched wire, upsetting the shanks thereof while cold, providing them with a cross-section greater than the wire, aging the rivets at a temperature of the order of about 300° F., and adjusting the temperature and the time of aging according to the analysis of alloy so as to produce such a temper that the rivets may be headed up without 10 becoming too brittle.

12. The process of manufacturing rivets from artificially aging aluminum alloys characterized by their low silicon content and non-spontaneous 15 aging comprising over 92% aluminum, .5% to 1% of nickel, .1% to 1% of copper, .25% to .5% chrome group metals and/or manganese and about .5% magnesium, which comprises making rivets of quenched wire, upsetting the shanks while cold to provide them with a greater cross-section than the wire, aging the rivets at a temperature of the order of about 300° F., and adjusting the temperature and the time of aging according to the analysis of the alloy so as to produce such a temper that the rivets may be headed 25 up without becoming too brittle.

13. The process of manufacturing rivets from artificially aging aluminum alloys characterized by their low silicon content and non-spontaneous 30 aging comprising making rivets of quenched wire of polygonal cross-section, upsetting the shanks while cold to provide them with a greater cross section than the wire, aging the rivets at a temperature of the order of about 300° F., and adjusting the temperature and time of aging and according to the analysis of the alloy so as to produce such a temperature that the rivets may be headed up without becoming too brittle.

14. The process of manufacturing rivets from 40 aluminum alloys of the class described characterized by the fact that the alloy has sufficient plasticity for riveting purposes after quenching and aging yet is deficient in shearing strength without work hardening by compression or upsetting which comprises increasing the cross-sectional area of the shank defining portion of 45 the rivet by at least 5% by an upsetting operation within a die whereby the shearing strength of the rivet is comparable with the upset heads of the rivet in use.

SVEN E. HYBINETTE.  
JUSTIN E. TINGAY.

#### CERTIFICATE OF CORRECTION.

Patent No. 2,062,977.

December 1, 1936.

SVEN E. HYBINETTE, ET AL.

It is hereby certified that error appears in the printed specification of the above numbered patent requiring correction as follows: Page 3, first column, line 17, claim 8, for "5%" read .5%; and that the said Letters Patent should be read with this correction therein that the same may conform to the record of the case in the Patent Office.

Signed and sealed this 2nd day of February, A. D. 1937.

(Seal)

Leslie Frazer  
Acting Commissioner of Patents.

by their low silicon content and non-spontaneous aging comprising over 92% aluminum, .5% to 1% of nickel, .1% to 1% of copper, .25% to .5% chrome group metals and/or manganese and 5 about .5% magnesium, which comprises the making of rivets from quenched wire, the shanks of such rivets having a cross-section greater than that of the wire, said greater cross-section being produced by upsetting while cold, and producing 10 such a temper by aging at a predetermined temperature for a predetermined time according to the analysis of the alloy, that the rivets may be headed up without becoming too brittle.

8. The process of manufacturing rivets from 15 artificially aging aluminum alloys characterized by their low silicon content and non-spontaneous aging comprising over 92% of aluminum, 5% to 1% of nickel, .1% to 1% of copper, .25% to .5% chrome group metals and/or manganese and 20 about .5% magnesium, which comprises the making of rivets from quenched wire, work hardening the shanks thereof by upsetting cold and producing such a temper by aging at a predetermined temperature for a predetermined time according 25 to the analysis of the alloy, that the rivets may be headed up without becoming too brittle.

9. The process of manufacturing rivets from artificially aging aluminum alloys characterized by their low silicon content and non-spontaneous 30 aging comprising over 92% of aluminum, .5% to 1% of nickel, .1% to 1% of copper, .25% to .5% chrome group metals and/or manganese and about .5% magnesium, which comprises the making of rivet blanks from quenched wire, upsetting 35 the same while cold, making rivets from such blanks and producing such a temper by aging at a predetermined temperature for a predetermined time according to the analysis of the alloy, that the rivets may be headed up without becoming too brittle.

10. The process of manufacturing rivets from artificially aging aluminum alloys characterized by their low silicon content and non-spontaneous aging comprising over 92% of aluminum, .5% to 45 1% of nickel, .1% to 1% of copper, .25% to .5% chrome group metals and/or manganese and about .5% magnesium, comprising forming a wire and upsetting said wire to form a rivet having a shank which has at least a 5% greater area of 50 cross-section than said wire from which the rivet is formed.

11. The process of manufacturing rivets from

artificially aging aluminum alloys characterized by their low silicon content and non-spontaneous aging comprising the making of rivets from quenched wire, upsetting the shanks thereof while cold, providing them with a cross-section greater than the wire, aging the rivets at a temperature of the order of about 300° F., and adjusting the temperature and the time of aging according to the analysis of alloy so as to produce such a temper that the rivets may be headed up without 10 becoming too brittle.

12. The process of manufacturing rivets from artificially aging aluminum alloys characterized by their low silicon content and non-spontaneous 15 aging comprising over 92% aluminum, .5% to 1% of nickel, .1% to 1% of copper, .25% to .5% chrome group metals and/or manganese and about .5% magnesium, which comprises making rivets of quenched wire, upsetting the shanks while cold to provide them with a greater cross-section than the wire, aging the rivets at a temperature of the order of about 300° F., and adjusting 20 the temperature and the time of aging according to the analysis of the alloy so as to produce such a temper that the rivets may be headed 25 up without becoming too brittle.

13. The process of manufacturing rivets from artificially aging aluminum alloys characterized by their low silicon content and non-spontaneous 30 aging comprising making rivets of quenched wire of polygonal cross-section, upsetting the shanks while cold to provide them with a greater cross-section than the wire, aging the rivets at a temperature of the order of about 300° F., and adjusting 35 the temperature and time of aging and according to the analysis of the alloy so as to produce such a temperature that the rivets may be headed up without becoming too brittle.

14. The process of manufacturing rivets from 40 aluminum alloys of the class described characterized by the fact that the alloy has sufficient plasticity for riveting purposes after quenching and aging yet is deficient in shearing strength without work hardening by compression or upsetting which comprises increasing the cross-sectional area of the shank defining portion of 45 the rivet by at least 5% by an upsetting operation within a die whereby the shearing strength of the rivet is comparable with the upset heads of the rivet in use.

SVEN E. HYBINETTE.  
JUSTIN E. TINGAY.

#### CERTIFICATE OF CORRECTION.

Patent No. 2,062,977.

December 1, 1936.

SVEN E. HYBINETTE, ET AL.

It is hereby certified that error appears in the printed specification of the above numbered patent requiring correction as follows: Page 3, first column, line 17, claim 8, for "5%" read .5%; and that the said Letters Patent should be read with this correction therein that the same may conform to the record of the case in the Patent Office.

Signed and sealed this 2nd day of February, A. D. 1937.

(Seal)

Leslie Frazer  
Acting Commissioner of Patents.

CERTIFICATE OF CORRECTION.

Patent No. 2,062,977.

December 1, 1936.

SVEN E. HYBINETTE, ET AL.

It is hereby certified that error appears in the printed specification of the above numbered patent requiring correction as follows: Page 3, first column, line 17, claim 8, for "5%" read .5%; and that the said Letters Patent should be read with this correction therein that the same may conform to the record of the case in the Patent Office.

Signed and sealed this 2nd day of February, A. D. 1937.

(Seal)

Leslie Frazer  
Acting Commissioner of Patents.